

## UNITED STATES PATENT OFFICE

2,015,345

## ALLOY

Robert H. Leach, Fairfield, Conn., assignor to  
Handy & Harman, New York, N. Y., a corpora-  
tion of New York

No Drawing. Application February 5, 1935,  
Serial No. 5,054

7 Claims. (Cl. 75—1)

This invention relates to alloys and is con-  
cerned more particularly with a novel alloy  
which is especially useful for brazing purposes.  
The new alloy has excellent physical properties,  
5 by virtue of which it can be employed to produce  
strong joints, and when used for brazing stain-  
less steel, it exhibits excellent resistance to cor-  
rosion resulting from certain types of chloride  
attack. Also, in certain forms, the alloy flows  
10 well at relatively low temperatures, a feature  
which enables the user to make strong joints  
with great facility.

The new alloy contains silver, copper, zinc,  
cadmium, and nickel, and the ranges of these  
15 ingredients are substantially as follows:

|         | Per cent |
|---------|----------|
| Silver  | 30-60    |
| Copper  | 12-35    |
| Zinc    | 5-20     |
| Cadmium | 5-20     |
| Nickel  | 1-5      |

Examples of specific compositions of the alloy  
which have been found to be satisfactory include  
25 the following, the analyses and the melting and  
flow points being approximate:

## Example No. 1

Per cent

|         |       |                        |
|---------|-------|------------------------|
| Silver  | 31.50 |                        |
| Copper  | 31.00 | Melting point 1180° F. |
| Zinc    | 16.50 | Flow point 1425° F.    |
| Cadmium | 19.00 |                        |
| Nickel  | 2.00  |                        |

## Example No. 2

|         |       |                        |
|---------|-------|------------------------|
| Silver  | 40.00 |                        |
| Copper  | 21.00 | Melting point 1180° F. |
| Zinc    | 18.00 | Flow point 1370° F.    |
| Cadmium | 19.00 |                        |
| Nickel  | 3.00  |                        |

## Example No. 3

|         |       |                        |
|---------|-------|------------------------|
| Silver  | 50.00 |                        |
| Copper  | 15.50 | Melting point 1195° F. |
| Zinc    | 15.50 | Flow point 1270° F.    |
| Cadmium | 16.00 |                        |
| Nickel  | 3.00  |                        |

## Example No. 4

|         |       |                        |
|---------|-------|------------------------|
| Silver  | 60.00 |                        |
| Copper  | 25.00 | Melting point 1315° F. |
| Zinc    | 8.00  | Flow point 1515° F.    |
| Cadmium | 6.00  |                        |
| Nickel  | 1.00  |                        |

The presence of the nickel within the range  
mentioned appears to be accountable for the in-  
creased corrosion resistance of the new alloy,  
10 and the optimum resistance to corrosion is ob-  
tained when the nickel is present in an amount  
of about 3%. The presence of the nickel in-  
creases the melting point, but, as shown by the  
foregoing examples, the proportions of the other  
15 ingredients of the alloy may be so selected as to  
give it a flow point as low as 1270°, which is  
sufficiently low for most purposes.

I claim:

1. An alloy which consists of silver from about  
30% to about 60%, copper from about 12% to  
about 35%, zinc from about 5% to about 20%,  
cadmium from about 5% to about 20%, and  
nickel from about 1% to about 3%.

2. An alloy which consists of silver from about  
30% to about 40%, copper from about 12% to  
about 35% zinc from about 5% to about 20%,  
cadmium from about 5% to about 20%, and  
nickel from about 1% to about 3%.

3. An alloy which consists of silver from about  
40% to about 50%, copper from about 12% to  
about 35%, zinc from about 5% to about 20%,  
cadmium from about 5% to about 20%, and  
nickel from about 1% to about 3%.

4. An alloy which consists of silver from about  
50% to about 60%, copper from about 12% to  
about 35%, zinc from about 5% to about 20%,  
cadmium from about 5% to about 20%, and  
nickel from about 1% to about 3%.

5. An alloy which consists of about 31.5% sil-  
ver, about 31% copper, about 16.5% zinc, about  
19% cadmium, and about 2% nickel.

6. An alloy which consists of about 40% sil-  
ver, about 21% copper, about 18% zinc, about  
19% cadmium, and about 2% nickel.

7. An alloy which consists of about 50% sil-  
ver, about 15.5% copper, about 15.5% zinc, about  
16% cadmium, and about 3% nickel.

ROBERT H. LEACH. 50

CERTIFICATE OF CORRECTION.

Patent No. 2,015,345.

September 24, 1935.

ROBERT H. LEACH.

It is hereby certified that error appears in the printed specification of the above numbered patent requiring correction as follows: First column, line 42, of Example No. 2, for "3.00" read 2.00; and that the said Letters Patent should be read with this correction therein that the same may conform to the record of the case in the Patent Office.

Signed and sealed this 5th day of November, A. D. 1935.

(Seal)

Leslie Frazer  
Acting Commissioner of Patents.